



US006354357B1

(12) **United States Patent**  
Clark

(10) **Patent No.:** US 6,354,357 B1  
(45) **Date of Patent:** Mar. 12, 2002

(54) **LOST FOAM METHOD OF CASTING A CYLINDER LINER WITH WATER JACKET**

5,960,851 A \* 10/1999 Donahue ..... 164/34

(76) Inventor: **Richark K. Clark**, 868 E. 1400 North Rd., Onarga, IL (US) 60955

\* cited by examiner

(\*) Notice: Subject to any disclaimer, the term of this patent is extended or adjusted under 35 U.S.C. 154(b) by 0 days.

*Primary Examiner*—Nam Nguyen  
*Assistant Examiner*—I. H. Lin  
(74) *Attorney, Agent, or Firm*—Kajane McManus

(21) Appl. No.: **09/298,892**

**ABSTRACT**

(22) Filed: **Apr. 26, 1999**

The lost foam method of casting a cylinder liner with water jacket comprises the steps of creating a blank identical to the liner desired, with a drain defined therein, from a heat-dissipated material such as styrofoam, coating the blank with core wash, placing the blank into a casting mold, filling the mold and a chamber defined within the blank with sand, pouring hot metal into the mold, extracting the formed metal liner from the mold, draining sand from within the chamber and plugging the sand drain.

(51) **Int. Cl.<sup>7</sup>** ..... B22C 9/02

**7 Claims, 6 Drawing Sheets**

(52) **U.S. Cl.** ..... 164/34; 164/45; 164/137

(58) **Field of Search** ..... 164/34, 45, 235, 164/246, 137, 340

(56) **References Cited**

**U.S. PATENT DOCUMENTS**

5,465,778 A \* 11/1995 Clark et al. ..... 164/137



**FIG. 1**

**FIG. 2**

**FIG. 3**

**FIG. 4**

**FIG. 6****FIG. 7****FIG. 5**



## LOST FOAM METHOD OF CASTING A CYLINDER LINER WITH WATER JACKET

### FIELD OF THE INVENTION

The present invention relates to a method of casting a cylinder liner with water jacket. More particularly, the method teaches the use of at least one styrofoam blank within a mold, the blank being identical in configuration to the cylinder liner cast with the method and defining a chamber therewithin which, when filled with sand prior to casting, will produce the passageway defining a circumferential water jacket. The method is applicable for use in both vertical and horizontal casting techniques.

### PRIOR ART

Heretofore, various methods of casting a cylinder liner with water jacket have been proposed. Also, casting may be accomplished in either a vertical or horizontal orientation.

Typically, such casting methods provide a mold which is multisectional, with the sections being positioned to define an air space between inner and outer mold sections which when filled with molten metal, define the cylinder liner. When it is desired to incorporate a water jacket into the liner, a complex core of solidified sand must be produced which, when suspended within the air space between the inner and outer mold sections, will not be replaced by the molten metal, thus creating a water path between inner and outer surfaces of the liner.

To accommodate suspension of such core, which may be of one or more sections, each section includes a plurality of radial arms which extend outwardly of the core and which must engage and be precisely supported by multiple outer sections of the mold for concentricity. This complexity of methodology requires the mold to be complex, of great precision, and therefore time consuming to arrange. It is thus inherently costly.

Further, cylinder liners are presently cast one at a time, due to complexity of the methodology used in creation thereof.

### SUMMARY OF THE INVENTION

Accordingly, a primary object of the present invention is to provide a simplified, and less costly, method of casting a cylinder liner with water jacket.

This object, as well as others, is accomplished by the method of the present invention wherein at least one foam blank conforming to the shape of the cylinder liner with water jacket is created and positioned within a mold, the blank including a circumferential cylindrical chamber therein and being coated with core wash, the mold and cylindrical chamber being filled with sand prior to introduction of molten metal into the mold, the molten metal replacing the foam blank, with the foam, dissipated by the heat of the metal, escaping from within the mold in the form of gas, with sand in the chamber being drained via a drain after cooling and removal of the casting, to define the water jacket flow path, with the drain being plugged after drainage of sand therethrough.

### BRIEF DESCRIPTION OF THE DRAWINGS

FIG. 1 is a perspective view of a cylinder liner with water jacket cast according to the method of the present invention, with internal structures thereof shown in phantom.

FIG. 2 is a cross sectional view through a mold containing at least one foam blank used in creating the cylinder liner of FIG. 1.

FIG. 3 is an identical cross sectional view through the foam blank of FIG. 2, showing the foam blank only.

FIG. 4 is a further cross sectional view through the foam blank taken at a diameter perpendicular to that of FIG. 3.

FIG. 5 is an enlarged cross sectional view through a sand drain port of the blank and is taken along line 5-5 of FIG. 4, and shows a cross section of a plug for the port.

FIG. 6 is a top plan view of the blank showing a first embodiment for the drain port and is taken along line 6-6 of FIG. 4.

FIG. 7 is a top plan view of the blank showing a second embodiment for the drain port and is taken along line 7-7 of FIG. 3.

FIG. 8 shows one top plan view of a sand filled mold with a plurality of blanks therein.

FIG. 9 shows another top plan view of a sand filled mold with a plurality of blanks therein.

### DESCRIPTION OF THE PREFERRED EMBODIMENT

Referring now to the drawings in greater detail, there is illustrated therein a cylinder liner with water jacket made in accordance with the teachings of the method of the present invention and generally identified by the reference numeral 10 (hereinafter referred to as liner 10).

As illustrated, the liner 10 includes an inner cylindrical wall 12 (shown in phantom) and an outer cylindrical wall 14. Between the walls 12 and 14 is defined a chamber 16 which serves as a water passageway, or water jacket, 16 of the liner 10. An entrance 18 into the water jacket 16 is provided at one suitable position and an exit therefrom (not shown) is provided at another suitable position so that there may be a flow of cooling water through the water jacket 16 and into a cylinder head (not shown) to be engaged thereupon.

Further, a plurality of air ports 22 are provided, girdling the liner 10 and extending through the walls 12 and 14 for intake of air by a piston (not shown) reciprocating within the cylinder defined by the inner wall 12, in known manner.

As stated above, creation of the liner 10 has heretofore been a complex, time consuming and expensive task.

Thus there has been a need for a simpler method of producing the liner 10 and it is believed the method of the present invention fills that need.

Referring now to FIGS. 2-9, there is illustrated therein, in its most simplistic form, the method and structures used in accomplishing the method.

Turning first to FIG. 2 for an overview of the simplified method, it will first of all be seen that a blank 24 is created which is an exact duplication of the liner 10 desired to be cast. The blank 24 may be made of any material which is similar to styrofoam in its characteristic of being dissipated by bubbling away at high temperatures.

The blank 24, in a preferred embodiment thereof is made of two sections 26 and 28, a first section 26 of which defines the inner cylindrical wall 12 of the liner 10 and a second section 28 which defines the outer wall 14 of the liner 10, with the sections 26 and 28 of the blank 24 being configured to define a longitudinal cylindrical chamber 30 therebetween, with the chamber 30 being intermittently interrupted by the presence of air throughports 32 girdling the blank 24 and extending from outside of the second section 28 through the first section 26 of the blank 24.

Although the preferred embodiment of the blank 24 is defined as being of two section construction, this is not to be construed as limiting.

Also, it will be understood that the entrance **18** and exit of the water jacket **16** need not be defined prior to casting, but may be provided by any suitable means such as drilling through an appropriate surface of the cast liner **10** to accommodate any required positioning thereof, as illustrated in FIG. 4, where the second section **28** of the blank **24** is shown to be uninterrupted.

Once the sections **26** and **28** are appropriately joined together, they are then coated almost completely, inside and out, with a coating **33** of a compound known as core wash which will not allow molten metal to seep therewith. Only desired points of ingress and egress are not coated.

For example, if vertical casting were selected, an upper wall **34** of the blank **24**, which is downwardly disposed for casting in this instance, would remain intermittently uncoated to produce an ingress for the metal in a bottom-up method.

One pattern of coating **33** is illustrated in FIG. 3, with the coating **33** being left off the remaining Figures for purposes of clarity.

With the method of the present invention wherein the coating **33** encases the blank **24**, a significant benefit is obtained which may not be readily apparent. In this respect, in methods of casting presently utilized, the liner **10** must necessarily undergo a significant amount of machining to have a functionally required configuration because a significant amount of excess metal is inherently present in such casting.

Such required machining is significantly reduced if not altogether eliminated by the present method because the blank **24**, in the first instance is identical in configuration to the desired liner **10** to be cast, and, in the second instance, with the coating **33** in place therearound, the metal will not seep past the barrier created by the coating **33**, the coating **33** also acting to reduce friction against which the metal is to flow, and therefore allowing the casting to be as near net size as possible. With the liner **10** being created near net size using the present method, it will be understood that any significant machining requirement is avoided.

The coated blank **24** is then inserted into a mold **40** which is of a significantly greater horizontal extent than the blank **24**, creating a void **42** around the blank **24**.

Further, as illustrated in the drawings, the blank **24** is inserted in a manner where a drain **44** leading into the chamber **30** faces upwardly. In the embodiment illustrated in FIG. 5, for use in vertical casting, the drain **44** is provided in what would be an underside **46** of the section **28** when righted.

It will be understood, however, that the drain **44** may also be provided at a radial point along an upwardly disposed portion of the circumference of the liner **10**, if the liner **10** where to be horizontally cast.

Considering the drain **44** in more detail, any suitable configuration thereof for use in filling/draining of the chamber **30** by sand **47** could be used.

In this respect, as illustrated in FIG. 6, the drain **44** could be defined as a circular channel **44** leading into the chamber **30**. Such circular channel **44** would be sealed off by engagement of a ring shaped plug **48** therewithin, the plug **48** being fixed to the liner **10** in any suitable manner, such as by welding. A cross section of such plug **48** is shown in FIG. 5.

Alternatively, the drain **44** could be defined as a radial array of spaced apart bores **44** as illustrated in FIG. 7, with each bore **44** being sealed with a plug **48**, a cross section of which is shown in FIG. 5, the plug **48** again being fixed to the liner **10** in any suitable fashion.

It will be understood that sealing of the drain **44**, in any workable embodiment thereof, would necessarily take place after the cooled casting of the liner **10** were removed from the mold **40**, righted, and drained of sand **47**.

Inasmuch as the blank **24** is necessarily identical to the liner **10** to be created therewith, it will logically follow that ports and channels will be provided in and on the blank **24** which are identical to those desired in the cast liner **10**.

It must be understood therefore that not only the exterior surfaces of the blank **24** but any surfaces past which molten metal fed into the ingress must not flow must also necessarily be coated with a coating **33** of core wash so as to remain open.

To the contrary end, so that the core wash coating **33** does not interfere with flow of molten metal to necessary areas, it is taught to engage any sections of the blank **24** together prior to dipping in or "coating" with core wash so that the core wash coating **33** does not adhere to the blank **24** at areas defining seams or points of juncture between sections of the blank **24**.

Summarizing, the foam blank **24** is created, core washed, and then seated within the mold **40** in a manner placing the drain **44** facing upwardly. Sand **47** is then poured into the mold **40** external and internal to the blank **24**, with the chamber **30** between the sections **26** and **28** of the blank **24** also being filled with sand **47** via the drain **44**. Molten metal is then delivered into the mold **40** in known manner, causing the styrofoam to dissipate from the bottom up through contact with the rising molten metal, which replaces the styrofoam.

Once the mold **40** is filled with molten metal, the metal is allowed to cool. After cooling, the formed metal liner **10** is removed from within the sand filled mold **40** and turned right side up, as shown in FIG. 1.

Once the liner **10** is righted, gravity takes over, drawing sand **47** out of the chamber **30** through the now downwardly directed drain **44**.

Once the sand **47** is removed, the drain **44** is plugged in the manner described above, producing the cylinder liner with water jacket **10**, the disclosed method being far simplified over previous methods of manufacture.

The simplicity of the method provides a further distinct advantage. It allows for a plurality of spaced apart blanks **24** to be received within an extended mold **40**, with a single sprue **50**, used in directing molten metal through the mold **40**, being capable of supplying the metal to the plurality of blanks **24**, as illustrated, in one embodiment, in FIG. 8, and in a further embodiment in FIG. 9.

Of course, it will be understood that the embodiments illustrated are best suited for vertical casting of the liner **10** and again should not be construed as limiting.

As described above the method of the present invention provides a number of advantages, some of which have been described above and others of which are inherent in the invention. Also, modifications may be proposed to the method without departing from the teachings herein. Accordingly the scope of the invention should only be limited as necessitated by the accompanying claims.

What is claimed is:

1. A method for casting a cylinder liner with water jacket comprising the steps of:  
creating a blank of heat-dissipated material substantially identical to the cylinder liner with water jacket to be cast, the blank including a drain therein;  
coating substantially all surface of the blank with core wash;

placing the blank inside a mold;  
 filling the mold, and a chamber defined within the blank  
 with sand;  
 pouring molten metal into the mold, the molten metal  
 dissipating and replacing the blank, thereby casting the  
 cylinder liner with water jacket;  
 waiting for the cast metal to cool;  
 removing the cast metal cylinder liner with water jacket  
 from the mold;  
 draining sand from the chamber within the cylinder liner  
 with water jacket via the drain; and  
 sealing the drain by suitably fixing a plug therein.

2. The method of claim 1 wherein a plurality of cylinder  
 liners are cast simultaneously.

3. The method of claim 1 wherein the heat dissipated  
 material is styrofoam.

4. The method of claim 3 wherein the styrofoam is in solid  
 form.

5. The method of claim 1 being suited for use in both  
 vertical and horizontal casting techniques.

6. A lost foam method for casting a cylinder liner with  
 water jacket comprising the steps of:  
 creating a blank of the cylinder liner with water jacket out  
 of styrofoam material with at least one sand drain  
 therein;  
 coating the blank with core wash;  
 placing the blank inside a mold;  
 filling the mold, and a chamber defined within the blank  
 with sand;

5

10

15

20

25

30

pouring molten metal into the mold to replace the styro-  
 foam blank therewith;  
 waiting for the metal to cool;  
 removing the created metal cylinder liner with water  
 jacket from the mold;  
 draining sand from the chamber within the cylinder liner  
 with water jacket via the drain; and  
 sealing the drain by suitably fixing a plug therein.

7. A lost foam method for casting a near net cylinder liner  
 with water jacket requiring significantly reduced if any  
 machining comprising the steps of:  
 creating a net blank of the cylinder liner with water jacket  
 out of styrofoam material with at least one sand drain  
 therein;  
 coating the blank with core wash;  
 placing the blank inside a mold;  
 filling the mold, and a chamber defined within the blank  
 with sand;  
 pouring molten metal into the mold to replace the styro-  
 foam blank therewith;  
 waiting for the metal to cool;  
 removing the created metal cylinder liner with water  
 jacket from the mold;  
 draining sand from the chamber within the cylinder liner  
 with water jacket via the drain; and  
 sealing the drain by suitably fixing a plug therein.

\* \* \* \* \*